

## UNITED STATES PATENT OFFICE.

ALFRED THAUSS, OF COLOGNE-DEUTZ, AND ALFRED GUENTHER, OF COLOGNE-RIEHL, GERMANY, ASSIGNEES TO GRASSELLI DYESTUFF CORPORATION, OF NEW YORK, N. Y., A CORPORATION OF DELAWARE.

## DYEING AND PRINTING PROCESS.

No Drawing. Application filed November 10, 1927, Serial No. 232,465, and in Germany December 3, 1926.

The present invention concerns the dyeing and printing of mixed fabrics containing wool and silk with dyestuffs to be employed in acid or neutral baths and consists in the 5 use of a sulfonation product obtained from resins.

In accordance with the present invention said mixed fabrics are subjected to a preliminary treatment with resins, as for example colophony, which have been rendered 10 soluble by means of sulfuric acid. The sulfonated resins behave in a like manner to that of sulfonated phenols, for example, and operate to reduce or prevent the absorption 15 of dyestuffs by wool and silk.

In some instances the addition of tin salts materially assists in obtaining the desired results.

The following examples will illustrate our 20 invention:—

*Example 1.*—A cotton material containing shoddy, which has been dyed fairly dark is to be dyed a most vivid marine blue color. The shoddy is first subjected to a preliminary 25 dyeing in an acid bath with most vivid dyestuffs, such as for example patent blue, alkali fast green, acid violet 4 B extra, the material is then rinsed and covered with a cotton dyestuff with the addition of the customary 30 amount of Glauber salt and 3% of colophony sulfonic acid at a temperature of about 50–60° C. According to the depth of the shade desired the dyeing can be effected with bright or black cotton dyestuffs. The addition 35 of the colophony sulfonic acid prevents the absorption of the cotton dyestuff by the shoddy whilst at the same time a much more vivid dyeing is obtained than is the case in the absence of colophony sulfonic acid.

*Example 2.*—In a wool material containing 40 threads of artificial silk for producing certain effects, the wool is subjected to a preliminary dyeing in an acid bath with the dyestuff obtained from benzaldehyde and ethyl-benzyl-metatoluidine-sulfonic acid; then the artificial silk is covered in a tepid 45 bath with 4% of the azo-dyestuff from benzidine-2-naphthylamino-5:7-disulfonic acid and 2-amino-5-naphthol-7-sulfonic acid with the addition of 3% of colophony sulfonic

acid. The two-fold color effect thus obtained is considerably more beautiful than would be the case without the addition of colophony sulfonic acid.

*Example 3.*—So-called half silk material, 55 which is composed of silk and cotton is dyed with the same dyestuffs and in a similar manner as described in Example 2. In this case also a far greater contrast effect is obtained than would be the case without the use of colophony sulfonic acid. 60

We claim:

1. In the process of dyeing and printing of mixed fabrics containing animal fibres with dyestuffs to be employed in acid or neutral 65 baths, the step which comprises the use of a sulfonation product obtainable from resins.

2. In the process of dyeing and printing of mixed fabrics containing animal fibres with dyestuffs to be employed in acid or neutral 70 baths, the step which comprises the use of colophony sulfonic acid.

3. In the process of dyeing and printing of mixed fabrics containing animal fibres with dyestuffs to be employed in acid or neutral 75 baths, the step which comprises the use of a sulfonation product obtainable from resins with the addition of tin salt.

4. In the process of dyeing and printing of mixed fabrics containing animal fibres with dyestuffs to be employed in acid or neutral 80 baths, the step which comprises the use of colophony sulfonic acid with the addition of tin salt.

5. In the process of reducing the absorptive power of animal fibres for acid or neutral dyeing dyestuffs the step which comprises adding a sulfonation product obtainable from resins to the dyebath. 85

6. In the process of reducing the absorptive power of animal fibres for acid or neutral dyeing dyestuffs the step which comprises adding colophony sulfonic acid to the dye-bath. 90

7. In the process of reducing the absorptive power of animal fibres for acid or neutral dyeing dyestuffs the step which comprises adding a sulfonation product obtainable from resins to the dyebath with the addition of tin salt. 95

8. In the process of reducing the absorptive power of animal fibres for acid or neutral dyeing dyestuffs the step which comprises adding colophony sulfonic acid to the 5 dyebath with the addition of tin salt.
9. The fibre treated with dyestuffs and sulfonation products obtainable from resins.

10. The fibre treated with dyestuffs and sulfonation products obtainable from resins and tin salt.

10  
In testimony whereof we have hereunto set our hands.

ALFRED THAUSS.  
ALFRED GUENTHER.